

June 26, 1928.

1,674,982

W. E. MOORE

ELECTRIC FURNACE AND METHOD OF CARBONIZING METALLIC CHARGES THEREIN

Filed May 11, 1922



Inventor

William E. Moore

By William L. Szymous

Attorney

## UNITED STATES PATENT OFFICE.

WILLIAM E. MOORE, OF PITTSBURGH, PENNSYLVANIA, ASSIGNOR TO PITTSBURGH RESEARCH CORPORATION, A CORPORATION OF DELAWARE.

## ELECTRIC FURNACE AND METHOD OF CARBONIZING METALLIC CHARGES THEREIN.

Application filed May 11, 1922. Serial No. 560,126.

This invention relates to metallurgical electric furnaces of the arc type, and more particularly to an improved method of carbonizing metallic charges in such furnaces.

5 It has heretofore been the common practice to construct the hearth or bottom of arc type metallurgical furnaces of refractory material, such as magnesite, dolomite or ganister, which becomes electrically conducting at high temperatures. It has also been proposed to construct furnace bottoms of this kind of a layer of refractory material which is of progressively increasing conductivity from the top downward.

10 Such a bottom, however, does not give the best results for certain classes of work, and I now propose to provide a furnace bottom consisting of a layer of substantially uniform high conductivity throughout. I 15 have also found that when treating such metals as iron or steel for the purpose of carbonizing them, it is desirable to form the furnace bottom or hearth of carbon or carbonaceous material capable of giving up 20 carbon to the charge.

The present invention also seeks to facilitate the carbonizing of a metallic charge by agitating the same while in contact with such a carbonaceous bottom or hearth, and 25 I have discovered that the carbonizing action can be expedited by mixing carbonaceous material with the charge and then agitating the charge while such material floats upon the surface thereof.

30 In order that the invention may be more readily understood, reference is had to the accompanying drawing forming a part of this specification and illustrating in vertical section a three phase furnace constructed in accordance with the invention and showing my improved means for agitating the charge.

Referring to the drawing in detail, the furnace is designated in its entirety by the reference numeral 1, and is shown as supported upon rockers 2 resting upon rollers 3 mounted on a concrete foundation 4. By virtue of this method of mounting, the furnace may be tilted so that the molten charge can be poured from the spout 5.

35 My improved furnace bottom consists of an outer shell 6 formed of metal plates, and a supporting layer 8 of refractory material such as basic or neutral brick, a lining 7

of suitable mortar being preferably interposed between the shell 6 and refractory layer 8.

The topmost or active layer 9, constituting the bottom or hearth of the furnace which is in direct contact with the charge, rests upon the layer 8, and consists of carbonaceous material such as carbon, or graphite, or a carbonaceous composition such as a mixture of graphite with ferro-alloys or other metals. This layer 9 constituting the bottom or hearth proper is of substantially uniform high conductivity throughout, and is electrically connected to the metallic shell 6 by means of a plurality of metal strips or fins 10 secured at one end to the shell 6, and having their other ends embedded in the layer 9 of carbonaceous material, such fins or strips extending through the refractory supporting layer 8.

The furnace is illustrated as having three electrodes *a*, *b* and *c*, extending through the roof as usual, and connected to the ends of the secondary winding of a three phase transformer *x*, *y*, the secondary winding *y* being star connected, and a conductor *z* extends from the neutral point of the star connected secondary to the metallic shell 6 of the furnace, being secured thereto by means of a suitable clip *z'*. Thus current not only passes from one electrode to the other, but may flow also from one or more of the electrodes through the furnace bottom.

When manufacturing and refining cast iron from iron or steel scrap or pig iron, it is often necessary to increase the percentage of carbon in the charge, that is, to carbonize it. I have found that one very effective way of doing this is to mix with the cold scrap when it is introduced into the furnace, a suitable amount of charcoal or coke. When the charge is melted this solid carbonaceous material floats on top of the molten charge and mixes with the impurities to form a carbonizing slag. I have found then, that when the charge is molten and in contact with the above described carbonaceous bottom or hearth at one side, and in contact with the carbonizing slag on the other side, it can be very effectively carbonized by agitating the liquid mass.

100 In the drawing 11 designates the molten

or liquid charge on which floats a slag 12 containing lumps of solid carbonizing material 13.

There are several ways in which this liquid charge can be agitated. Thus, for example, fairly good results can be obtained by simply thrusting a pole of green wood into the charge, the heat of the charge immediately vaporizing the volatile constituents of the wood, thus causing ebullition of the molten mass.

A more effective method, however, is to plunge into the molten charge the end of a pipe 14, such end being of course protected 15 by asbestos or other heat insulating material, as indicated at 15, and then introducing into the charge through the pipe 14 and attached hose 16, a non-oxidizing fluid. The pipe may be inserted into the furnace 20 through the opening 18 adjacent the pouring spout, which opening is closed by the usual door 19. The fluid employed may be either a non-oxidizing or reducing gas such as hydrogen, under pressure, or it may 25 be in the nature of a hydrocarbon, either gaseous or liquid. In either case the passage of the gases or vapors through the molten charge produces a violent bubbling or ebullition, thus agitating the mass and 30 bringing all parts thereof into intimate contact with both the carbonaceous bottom and the carbonizing slag.

Moreover, if a hydrocarbon or oil is employed the gases or vapors therefrom fill 35 the space in the furnace above the charge and themselves constitute carbonaceous or carbonizing material. Thus by using a fluid hydrocarbon for bubbling through the charge, it performs the double function of 40 agitating the molten mass and at the same time supplying carbon which may be absorbed by the charge.

It will therefore be understood that I contemplate carbonizing a metallic charge in 45 any one of the several ways mentioned or by employing all of the several methods at the same time. Thus I may omit the solid carbonaceous material and produce the carbonizing simply by agitating the molten mass 50 in contact with my improved carbonaceous hearth, or I may agitate the mass by means of a fluid hydrocarbon as described, or I may use an inert gas and employ solid carbonizing material in the form of a supernatant 55 slag.

In addition to its carbonizing function, my improved carbonaceous bottom is found to be highly resistant to both acid and basic slags.

60 What I claim is:

1. In the treatment of iron and other metals in an arc type electric furnace, the method of carbonizing the charge which consists in mixing therewith carbonaceous 65 materials, heating until molten, and then

agitating the mixture of carbonaceous material and molten metal.

2. In the treatment of iron and other metals in a direct arc type electric furnace, the method of carbonizing the charge which 70 consists in melting it when in contact with carbonaceous material and agitating the molten mass while still in contact with the carbonaceous material by bubbling there-through a hydrogen containing gas. 75

3. In the treatment of iron and other metals in an arc type electric furnace, the method of carbonizing the charge which 80 consists in melting it when in contact with carbonaceous material and agitating the molten mass while still in contact with the carbonaceous material by bubbling there-through a reducing gas.

4. In the treatment of iron and other metals in an arc type electric furnace, the 85 method of carbonizing the molten charge which consists in introducing into the furnace and plunging beneath the surface of the molten charge a pipe having a heat insulated end, and forcing through such 90 pipe into the charge suitable quantities of fluid hydrocarbons.

5. In the treatment of iron and steel in an arc type electric furnace, the method of carbonizing which consists in introducing 95 lumps of carbonaceous material into the furnace with the cold charge, melting down the charge, and then agitating the molten charge while the carbonaceous material floats on the surface thereof. 100

6. In the treatment of iron and steel in an arc type electric furnace, the method of carbonizing which consists in introducing into the furnace carbonaceous material of such a nature that it floats on top of the 105 molten charge, and then agitating such charge by causing to bubble therethrough a non-oxidizing fluid.

7. In the treatment of iron and steel in an arc type electric furnace having a hearth or bottom of carbonaceous material, the method which consists in agitating the molten charge by plunging into the same from above a piece of pipe having a heat insulated end, and forcing therethrough a non-oxidizing fluid which bubbles up through the charge while the charge is in contact with the carbonaceous hearth. 115

8. In the treatment of iron and steel in an arc type electric furnace having a hearth or bottom of carbonaceous material, the method which consists in introducing into the furnace carbonaceous material of such a nature that it floats on top of the molten charge, and then agitating such charge while it is 120 in contact with both the carbonizing hearth and the supernatant carbonaceous material. 125

In testimony whereof I affix my signature.

WILLIAM E. MOORE.